

# UNITED STATES PATENT OFFICE.

CARLETON ELLIS, OF LARCHMONT, NEW YORK, ASSIGNOR TO CHADELOID CHEMICAL COMPANY, OF NEW YORK, N. Y., A CORPORATION OF WEST VIRGINIA.

## FINISH-REMOVER.

1,147,851.

Specification of Letters Patent. Patented July 27, 1915.

No Drawing.

Application filed September 27, 1907. Serial No. 394,917.

To all whom it may concern:

Be it known that I, CARLETON ELLIS, a citizen of the United States, and resident of Larchmont, in the county of Westchester 5 and State of New York, have made certain new and useful Inventions Relating to Finish-Removers, of which the following is a specification.

This invention relates to finish removers 10 and the processes of making the same and relates especially to removers comprising chlorinated or other compounds having an acid tendency in which antacid materials are so incorporated as to be non-settling and 15 to obviate or correct such tendency.

Chlorinated organic solvents, such as carbon tetrachlorid, chlor benzol, chlor toluol, acetylene chlorid and so forth, are desirable 20 as ingredients for paint or varnish removers because reducing or destroying their inflammable character. Such remover ingredients have in some cases an acid tendency, that is, either possess acid properties or have a tendency to form bodies of an undesirable acid character in connection with 25 the ordinary alcoholic or other remover ingredients, as is also sometimes the case with other esterification products containing chlorin or other acid radicals. Effective 30 antacid material is desirable in removers of this character to prevent or neutralize such acid tendency and should be thoroughly and uniformly incorporated with the other remover ingredients and be of a non-settling 35 character in order to be most effective. Soaps of the fatty acids, such as sodium, potassium or ammonium stearate, palmitate, oleate, resinate, and so forth, are desirable 40 non-settling antacid materials if properly incorporated in the remover which can be readily accomplished by thoroughly drying the soap and then dissolving it in hot alcohol, preferably after its pulverization and 45 then incorporating the chlorinated or other penetrating solvents. Antacid material of this character may be used in removers in connection with loosening finish solvents, that is, solvents having a generally alcoholic 50 character or action in removers, such, for example, as methyl, ethyl, amyl, allyl, and denatured alcohols, acetone, methyl acetone, methyl ethyl ketone, acetone oil, light oil of hard wood tar, butyrene and allied solvents.

In addition to the chlorinated finish solvents referred to other penetrating finish solvents, that is, solvents having a generally benzolic character or action in removers may be employed, including benzol, toluol xylol, cumene, benzin and other petroleum hydrocarbons and methyl, ethyl, amyl and other ethers and esteric compounds. Although not necessary in all cases suitable stiffening material may be employed, such as flour, starch, wood flour, whiting, infusorial earth 65 and also film-forming stiffening material may be employed, such as waxes or waxy material, nitrated cellulose and other solid organic bodies having the property of forming evaporation retarding films on the removers. An illustrative remover of this character may be prepared by thoroughly drying a good sodium soap, such as a good grade of tallow or olive oil soap, by drying 70 for several hours at a temperature of about 110° C., grinding the soap to a fine powder when it is sufficiently dried for this purpose, and then thoroughly drying the soap powder. A quantity of this dried soap 75 powder and a quantity of denatured alcohol 80 may be put into a receptacle provided with a reflux condenser and boiled until the alcohol is saturated with the soap. 5 parts of this alcohol soap solution may be diluted with 5 parts of denatured alcohol and the 85 resulting solution mixed with 9 parts of carbon-tetrachlorid in which 1 part of cere- 90 sin has been dissolved, the various ingredients being, of course, thoroughly incorporated by agitation in a suitable stirrer or otherwise.

This invention has been described in connection with a number of illustrative ingredients, formulas, proportions and processes, to the details of which disclosure the invention is not, of course, to be limited.

What is claimed is:—

1. The finish remover comprising approximately 5 parts of denatured alcohol which has been saturated with dried powdered sodium soap and incorporated with 5 parts of denatured alcohol and 9 parts of carbon-tetrachlorid in which 1 part of cere- 100 sin wax has been dissolved.

2. The finish remover comprising approximately 5 parts of denatured alcohol in which soapy antacid material has been thoroughly dissolved and with which are incor- 105

porated 5 parts of loosening finish solvent material, and 9 parts of chlorinated solvent material and waxy stiffening material.

3. The substantially fluent non-aqueous finish remover comprising approximately five parts of alcohol in which soapy antacid material has been dissolved and with which are incorporated five parts of loosening finish solvent material and nine parts of chlorinated solvent material and stiffening material.

4. The finish remover consisting substan-

tially of volatile finish solvent material comprising loosening finish solvent material in which soapy antacid material has been dissolved and with which approximately equal proportions of penetrating solvent material including a chlorinated solvent has been incorporated.

15

CARLETON ELLIS.

Witnesses:

HARRY L. DUNCAN,  
JESSIE B. KAY.